# EUROPEAN PATENT SPECIFICATION

(11) **EP 3 679 177 B1**
(45) Date of publication and mention of the grant of the patent: **06.11.2024**
(21) Application number: 18853747.6
(22) Date of filing: 07.09.2018
(51) Int. Cl.: C25B 3/07, C25B 3/25, C25B 3/26, C25B 11/052, C25B 11/089, C25B 11/091

(54) **BINARY ALLOYS AND OXIDES THEREOF FOR ELECTROCATALYTIC REDUCTION OF CARBON DIOXIDE**
BINÄRE LEGIERUNGEN UND IHRE OXIDE ZUR ELEKTROKATALYTISCHEN REDUKTION VON KOHLENDIOXID
ALLIAGES BINAIRES ET LEURS OXYDES POUR LA RÉDUCTION ÉLECTROCATALYTIQUE DU DIOXYDE DE CARBONE

(30) Priority: 07.09.2017 US 201762555503 P; 22.03.2018 US 201862646816 P
(43) Date of publication of application: 15.07.2020
(73) Proprietor: The Trustees of Princeton University, Princeton, NJ 08544 (US)
(72) Inventor: BOCARSLY, Andrew, Plainsboro NJ 08536 (US); PARIS, Aubrey, Delran NJ 08075 (US); FRANCIS, Sonja, A., Princeton NJ 08540 (US); CHU, An, Amherst MA 01002 (US)
(74) Representative: Greenwoods
(86) International application number: PCT/US2018/050016
(87) International publication number: WO 2019/051268

(56) References cited:
- US-A- 5 747 185
- US-A1- 2013 206 608
- US-A1- 2014 206 895
- US-A1- 2015 152 564
- WATANABE ET AL.: "Design of Alloy Electrocatalysts for C02 Reduction III. The Selective and Reversible Reduction of C02 on Cu Alloy Electrodes", JOURNAL OF THE ELECTROCHEMICAL SOCIETY, vol. 138, no. 11, 1991, pages 3382 - 3389, XP055580999
- TORELLI ET AL.: "Nickel-Gallium-Catalyzed Electrochemical Reduction of C02 to Highly Reducec Products at Low Overpotentials", ACS CATALYSIS, vol. 6, no. 3, 17 February 2016 (2016-02-17), pages 2100 - 2104, XP055581003
- IKEDA ET AL.: "Selective Formation of Formic Acid, Oxalic Acid, and Carbon Monoxide by Electrochemical Reduction of Carbon Dioxide", BULLETIN OF THE CHEMICAL SOCIETY OF JAPAN, vol. 60, July 1987 (1987-07-01), pages 2517 - 2522, XP055581008
- RAMI ET AL.: "Kinetics of hydrogen evolution on Ni-AI alloy electrodes", JOURNAL OF APPLIED ELECTROCHEMISTRY, vol. 22, 1992, pages 376 - 382, XP055581010
- CHERIAN ET AL.: "Oxidative dehydrogenation of propane over Cr2O3/Al2O3 and Cr203 catalysts: effects of loading, precursor and surface area", APPLIED CATALYSIS A, vol. 233, 10 July 2002 (2002-07-10), pages 21 - 33, XP004367101, DOI: doi:10.1016/S0926-860X(02)00132-1
- ZHU ET AL.: "Recent Advances in Inorganic Heterogeneous Electrocatalysts for Reduction of Carbon Dioxide", ADVANCED MATERIALS, vol. 28, 21 March 2016 (2016-03-21), pages 3423 - 3452, XP055581016
- "Electrostatic induction", WIKIPEDIA, 17 June 2017 (2017-06-17), pages 1 - 5, XP055581021, Retrieved from the Internet <URL:https://en.wikipedia.org/w/index.php?title=Electrostatic_induction&oldid=786094093> [retrieved on 20181110]

## Description

### STATEMENT OF GOVERNMENT RIGHTS

This invention was made with government support under Grant No. CHE1308652 awarded by the National Science Foundation. The government has certain rights in the invention.

### FIELD

The present invention relates to the electrocatalytic reduction of CO₂ and, in particular, to the electrocatalytic reduction of CO₂ to produce oxygenated organic products.

### BACKGROUND

Global atmospheric CO₂ concentrations have risen continuously for the past two centuries largely due to anthropogenic activities such as fossil fuel combustion, industrial manufacturing, and land clearing. This is cause for alarm because effects of high CO₂ levels include changes in water availability and food production capacity as well as implications for human health. The burning of fossil fuels not only sustains high CO₂ levels, but it also reduces our access to compounds which are critical chemical feedstocks. The electrochemical transformation of CO₂ into chemical feedstocks and energy sources offers a potential solution to this far-reaching problem, effectively turning a societal hindrance into practical products. Electrochemical transformation of CO₂ is shown for example in:-
WATANABE et al.: "Design of Alloy Electrocatalysts for CO2 Reduction III. The Selective and Reversible Reduction of CO2 on Cu Alloy Electrodes", Journal of the Electrochemical Society, vol. 138, no. 11, 1991, pages 3382-3389;
TORELLI et al.: "Nickel-Gallium-Catalyzed Electrochemical Reduction of CO2 to Highly Reduced Products at Low Overpotentials", ACS Catalysis, vol. 6, no. 3, 17 February 2016 (2016-02-17), pages 2100-2104;
IKEDA et al.: "Selective Formation of Formic Acid, Oxalic Acid, and Carbon Monoxide by Electrochemical Reduction of Carbon Dioxide", Bulletin of the Chemical Society of Japan, vol. 60, July 1987 (1987-07), pages 2517-2522;
US 2014/206895 A1.
US 2015/152564 A1 discloses a formic acid generation apparatus for generating formic acid by reducing carbon dioxide, the apparatus comprising a cathode electrode having a gallium oxide region on a surface thereof. The gallium oxide region may be doped.

### SUMMARY

The present invention provides a system and method for providing oxygenated organic products asset out in the claims.

Embodiments are described in more detail in the following detailed description.

### BRIEF DESCRIPTION OF THE DRAWINGS

FIG. 1 provides powder X-ray diffraction of Ni₃Al film (not encompassed by the wording of the claims) on glassy carbon referenced to PDF 01-071-5883. Scanning electron microscopy (SEM) images of the Ni₃Al film are also provided on the right side.
FIG. 2(A) are cyclic voltammograms obtained using Ni₃Al (not encompassed by the wording of the claims) on glassy carbon under CO₂ (red) and Ar (black). Voltammograms were obtained at a scan rate of 100 mV/s with Pt mesh counter and Ag/AgCl reference electrodes in 0.1 M K₂SO₄ at pH 4.5.
FIG. 2(B) provides ¹H-NMR of 0.1 M K₂SO₄ electrolyte solution following bulk electrolysis at -1.38 V, indicating the presence of 1-propanol, methanol, and formate as major products. The broad peak at 4.66 ppm is a suppressed water signal, and all peaks are referenced to a 1,4-dioxane internal standard.
FIG. 2(C) provides ¹³C-NMR confirming the presence of ethanol.
FIG. 2(D) provides ¹H-¹³C HSQC indicating that ¹³C-labelled acetone was produced.
FIG. 3(A) - Faradaic efficiencies for CO, 1-propanol, methanol, and formate are reported at a range of applied potentials.
FIG. 3(B) - Faradaic efficiencies for H₂, CO, and liquid products are plotted as a function of pH and confirm charge balance (top); the liquid product distribution is provided in the lower portion of panel (B).
FIG. 4 quantifies the major liquid products, 1-propanol and methanol, plotted versus the amount of charge passed using (A) CO₂ and (B) CO feedstocks.
FIG. 5A presents an XRD pattern (left) of Cr₂O₃-Ga₂O₃ referenced to Cr₂O₃ (PDF 00-038-1479) and Ga₂O₃ (PDF 01-074-1610); and an SEM image (right) of Cr₂O₃-Ga₂O₃ platelets.
FIG. 5B is a fitted XPS spectra of Cr (left) and Ga (right), indicating that the surface is primarily made up of metal oxides. Peaks were referenced to adventitious carbon at 284.5 eV (not shown).
FIG. 6 is an IR spectrum of calcium oxalate derived from Cr₂O₃-Ga₂O₃ mediated electrolysis, confirming that oxalate is a CO₂ reduction product.
FIG. 7 illustrates pH dependence of Faradaic efficiencies for carbon-containing products. Experiments were performed at -1.38 V vs. Ag/AgCl using CO₂-saturated 0.1 M KCl buffered with KHCO₃ (pH > 4) or adjusted with HCl (pH < 4).
FIG. 8 illustrates potential dependence of Faradaic efficiencies for carbon-containing products. Experiments used pH 4.05, 0.1 M KCl electrolyte, and all potentials tested were more positive than the thermodynamic potential for one-electron reduction of CO₂. Optimal oxalate production was achieved at -1.48 V vs. Ag/AgCl.
FIG. 9 illustrates Faradaic efficiencies of carbon-containing products. While oxalate generation is suppressed at high KCl concentrations, low CO and high formate Faradaic efficiencies contribute to decreased oxalate production at low KCl concentrations. Electrolyses were performed at -1.48 V vs. Ag/AgCl.
FIG. 10 illustrates Faradaic efficiencies of carbon-containing products. Cr-rich stoichiometries result in the lowest efficiencies for CO. Electrolyses were performed at -1.48 V vs. Ag/AgCl in 0.1 M KCl (pH 4.1).

### DETAILED DESCRIPTION

Embodiments described herein can be understood more readily by reference to the following detailed description and examples and their previous and following descriptions. It should be recognized that these embodiments are merely illustrative of the principles of the present invention. Numerous modifications and adaptations will be readily apparent to those of skill in the art without departing from the scope of the invention.

In the following, systems employing oxides of binary alloys for the electrocatalytic reduction of CO₂ to various organic products are described. Binary alloys and/or oxides thereof suitable for electrocatalytic reduction of CO₂ may comprise a transition metal and a post-transition metal (TM/PTM). The transition metal may be a first row transition metal. Moreover, post-transition metals can be selected from Groups IIB-VA of the Periodic Table. Groups of the Periodic Table referenced herein are identified according to the CAS designation. Binary alloys, may be of the formula TMₓPTM_{y}, wherein x and y are integers independently selected from 1 to 10. Transition metal and post-transition metal can be combined in any ratio operable for the electrocatalytic reduction of CO₂ into various organic products. For example, x may be 3 and y may be 1. Also, x can range from 1 to 9 and y can range from 1 to 6. Table I provides a listing of various binary alloys operable for the electrocatalytic reduction of CO₂ into various organic products, including oxygenated products comprising two or more carbon atoms and/or two or more oxygen atoms.

**Table I - TMₓPTM_{y}, wherein x = 3 and y =1**

| |
|---|
| Ni-Al (not encompassed by the wording of the claims) |
| Ni-Ga (not encompassed by the wording of the claims) |
| Ni-In (not encompassed by the wording of the claims) |
| Cu-Al (not encompassed by the wording of the claims) |
| Fe-Ga (not encompassed by the wording of the claims) |
| Fe-Al (not encompassed by the wording of the claims) |
| Mn-Al (not encompassed by the wording of the claims) |
| Mn-Ga (not encompassed by the wording of the claims) |
| Co-Al (not encompassed by the wording of the claims) |
| Ni-Zn (not encompassed by the wording of the claims) |
| Co-Ga (not encompassed by the wording of the claims) |
| Cr-Al (not encompassed by the wording of the claims) |
| Cr-Ga (as an oxide, encompassed by the wording of the claims) |
| Ag-Al (not encompassed by the wording of the claims) |
| Ag-Ga (not encompassed by the wording of the claims) |

As claimed, the binary alloy is in oxide form. Binary metal oxides, for example, may form surface and/or bulk regions of the material administering the electrocatalytic reduction of CO₂. The working electrode comprises the binary system of chromium oxide and gallium oxide including, but not limited to, Cr₂O₃-Ga₂O₃. Moreover, stoichiometries or ratios of the transition metal and post-transition metal can remain the same in the metal oxide as in the binary alloy. Accordingly, the values provided for x and y above apply to the metal oxide. In the claimed chromium oxide-gallium oxide, the ratio of chromium to gallium can be 3:1.

The chromium oxide-gallium oxide can be provided as a thin film on the working electrode of the electrochemical cell. The thin film can be deposited on any substrate consistent with the objectives of the present invention. In some embodiments, for example, the thin film of alloy and/or oxide is deposited on glassy carbon.

The electrochemical cell also comprises an electrolyte solution having CO₂ dissolved therein. Any electrolyte solution consistent with the objectives of the present invention can be employed, including aqueous electrolyte solution. In some embodiments, aqueous electrolyte solution comprises alkali metal salt or alkaline earth metal salt. The electrolyte solution may also comprise CO in addition to CO₂, in some embodiments. The electrolyte solution can have neutral or acidic pH, in some embodiments. The electrolyte solution, for example, can have pH ranging from 3-7 or from 3-6.5. In other embodiments, pH of the electrolyte solution ranges from 4-6. Oxygenated organic products formed by the electrocatalytic reduction of CO₂ at the working electrode can include one or more of propanol, butanol, ethanol, oxalate, formic acid or formate and acetone. In some embodiments, oxygenated products include a single oxygen atom, such as CO and methanol.

The oxides of the working electrode are operable to form additional organic products from the electrocatalytic reduction of CO₂. These organic products can comprise one carbon atom, two carbon atoms, three carbon atoms or mixtures thereof. Such organic products can be aliphatic or oxygenated.

In another aspect, a system for providing oxygenated organic products comprises an electrochemical cell including an electrolyte solution comprising CO₂, and an electrode comprising a mixture of metal oxides. The electrode comprises an electrocatalytic site for reduction of CO₂ to CO, wherein CO is incorporated into the oxygenated organic products. The a mixture of metal oxides, comprises chromium oxide and gallium oxide. The electrocatalytic site for reduction of CO₂ to CO may be anionic or exhibit anionic character, in some embodiments. Additionally, the electrocatalytic site may be selective to the reduction of CO₂ to CO in that the site does not participate in other redox chemistries. The electrode may contain one or more additional electrocatalytic sites for producing other products. In some embodiments, for example, the electrode comprises a non-ionic site for the production of formate in addition to the electrocatalytic site for CO₂ reduction to CO.

These embodiments are further illustrated in the following non-limiting examples.

### Comparative EXAMPLE 1 (not encompassed by the wording of the claims) - Ni₃Al Electrocatalytic Reduction of CO₂ to Oxygenated Organics

Here it is shown that a Ni₃Al thin film electrocatalyst supported on glassy carbon can generate reduced C₁, C₂, and C₃ products from CO₂ with good performance, stability, and reproducibility at modest overpotential. Competing copper-based electrocatalysts were first reported to carry out the reduction of CO₂ to C₂ and C₃ products in 1988. For the first time it is demonstrated that metal alloys can generate C₃ products, electrocatalytic activity that, until now, has been uniquely associated with copper-based electrode systems. Further, the data presented here suggest that the Ni₃Al system is more stable than copper-based systems.

Ni₃Al thin film alloys were synthesized on glassy carbon substrates by adapting a drop-casting and furnace reduction procedure employed by Torelli et al., ACS Catal. 2016, 6, 2100-2104. As shown in FIG. 1, powder X-ray diffraction of the alloys confirmed the successful generation of the cubic Ni₃Al composition as indicated by the (111) and (211) planes; energy-dispersive X-ray spectroscopy supported the compositional analysis. X-ray photoelectron spectra (XPS) of a virgin (i.e. not utilized) electrode showed the presence of three Ni species: Ni(OH)₂, NiO, and Ni metal, with the Ni²⁺ components making up a majority of the composition, while all surface Al adopted the oxidized Al₂O₃ form. Thin films exhibited macroscopic surface areas of approximately 0.75 cm², while imaging by scanning electron microscopy, shown in FIG. 1, indicated that the films were comprised of micro-scale platelets uniformly distributed across the glassy carbon surface. In preliminary electrochemical experiments, cyclic voltammetry scans performed in aqueous electrolyte under CO₂ versus Ar saturation resulted in relatively featureless traces, although current enhancement was observed at more negative potentials leading into a proton reduction wave (FIG. 2A).

Bulk electrolysis experiments using the Ni₃Al thin film on glassy carbon as the working electrode and a Pt mesh counter electrode were performed at an applied potential of -1.38 V vs. Ag/AgCl in a sealed two-compartment cell containing 0.1 M K₂SO₄ electrolyte solution saturated with CO₂ (pH 4.5). Total current densities of -2.1 ± 0.4 mA/cm² were recorded and could be maintained for a period of several hours. ¹H-NMR spectra obtained as a function of electrolysis time (see FIG. 2B) indicated the growth of largely isolated peaks characteristic of 1-propanol (triplet; 0.73 ppm), acetone (singlet; 2.07 ppm), ethanol (triplet; 1.03 ppm), methanol (singlet; 3.20 ppm), and formate (singlet; 8.29 ppm) over time.

Several analytical methods were employed to confirm the identities of these C₁-C₃ products and to support the assertion that they were, in fact, derived from the CO₂ starting material. Electrolysis experiments performed using ¹³CO₂ yielded ¹H-NMR traces for 1-propanol, ethanol, methanol, and formate exhibiting the peak splitting expected for ¹³C-coupling. However, a large doublet signal of 2-propanol (believed to be generated from acetone reduction) obscured the ethanol triplet, and acetone splitting was inconclusive using simple ¹H-NMR. To resolve these ambiguities ¹³C-NMR spectra were obtained, resulting in the observation of a clear set of ethanol peaks (FIG. 2C). In addition, a ¹H-¹³C heteronuclear single quantum correlation (HSQC) NMR experiment was performed to confirm the presence of ¹³C-labelled acetone (FIG. 2D). Moreover, peak splitting within the ¹³C-NMR spectrum, particularly in the C₂ and C₃ products, implied that all product carbon atoms were derived from the original ¹³CO₂ material. Mass spectrometry further supported the NMR results.

Faradaic efficiencies of 1.9 ± 0.3% for 1-propanol, 1.0 ± 0.2% for methanol, and 0.75 ± 0.03% for formate were observed, with lesser contributions from ethanol and trace amounts of acetone. As shown in FIG. 3A, the potential dependence of CO₂ electroreduction to these liquid products confirms -1.38 V vs. Ag/AgCl as the optimal potential at which to operate the electrochemical cell. The electrolyte pH was also found to strongly impact the overall CO₂ conversion efficiency and the distribution of products as summarized in FIG. 3B. Highest product yields were observed at pH~4.5. It is worth noting that the solution pH changes at most a few tenths of a unit from the beginning to the end of an electrolysis experiment. Given that all electrolysis experiments utilized efficient and continuous stirring of the electrolyte, the constant bulk value of the electrolyte pH suggests that any pH variation at the electrode surface was slight and, according to FIG. 3B, did not drastically alter the product distribution.

An understanding of the mechanism facilitated by the Ni₃Al film would allow for future work in optimizing the generation of select C₁, C₂, or C₃ products. As such, the headspace of the electrochemical cell following electrolysis was examined, and it was discovered that CO was the only gaseous CO₂ reduction product generated. Like the liquid products, CO production was maximized at -1.38 V vs. Ag/AgCl, at which point Faradaic efficiencies of 33 ± 3% were attained. As reported in FIG. 3B, the remainder of the gas generated was H₂. The fact that maximum liquid product and CO yields are achieved at the same applied potential suggests that CO might be an intermediate in CO₂ electroreduction to major products such as 1-propanol and methanol. To test this hypothesis, CO₂ was replaced with CO as the feedstock in electrolysis and examined the resulting reduction products by ¹H- NMR. Ni₃Al thin films on glassy carbon reduced CO to methanol as well as the C₂ and C₃ liquid products achieved using a CO₂ feedstock and in the same relative quantities. Electrolysis experiments utilizing a mixed ¹³CO₂/¹²CO feedstock indicated that 1-propanol, methanol, ethanol, and acetone were preferentially generated from CO, with only small contributions from ¹³CO₂. In these experiments, trace or no formate was produced.

Furthermore, plotting 1-propanol and methanol quantities obtained during CO-feedstock trials against the amount of charge passed during an experiment, as shown in FIGS. 4A and 4B, illuminated differences in rate of product generation. Specifically, when the electrochemical cell was saturated with CO₂, both 1-propanol and methanol increased linearly with charge passed. However, when the feedstock was switched to CO, though 1-propanol retained its linearity (but had a slope that was greater by two orders of magnitude than that of the CO₂-derived analog), methanol formation adopted an exponential growth curve.

Accordingly, it appears that CO is, in fact, an intermediate leading to Ni₃Al's generation of methanol, C₂, and C₃ products from CO₂. It is suggested that the reduction of CO₂ to CO is the limiting process in this electroreduction, leading to preferential use of CO as the reactant when both CO and CO₂ are present, as well as linear product generation curves when CO₂ is the available species being reduced. Only one CO₂ molecule, and therefore one CO molecule, must be present to produce methanol, so when the system is supplied with CO as the feedstock it generates methanol relatively easily, leading to an exponential production curve. The generation of 1-propanol necessitates the presence of three carbon atoms, so even if the limiting step is removed by providing CO as the reactant, accumulation of three CO molecules near one another on the thin film surface is still required. Thus, the linear trend for 1-propanol remains, though its slope increases because the CO₂ to CO conversion step has been eliminated. This sort of mechanistic analysis, though preliminary, will help to improve the design and optimization of future alloy catalysts.

The fact that Ni₃Al generates quantifiable amounts of C₃ products, alongside useful C₁ and C₂ products, is interesting because of the thin film's stability, reproducibility, and modest overpotential. It is worth noting that, upon cursory examination of the related intermetallic NiAl, significantly diminished Faradaic efficiencies were achieved for the products described herein. The previously reported Ni-Ga thin film system plated on a highly oriented pyrolytic graphite substrate achieved maximum Faradaic efficiencies for C2 products of approximately 1.7% and 0.4% for ethane and ethylene, respectively, with no indication of C3 product formation. Methane was also observed. Faradaic efficiency of 1.9 ± 0.3% for the C₃ product 1-propanol indicates a heterogeneous synthetic route to higher order organic compounds that has not previously been reported at alloy electrode interfaces.

The inventors have recently suggested a catalytic efficiency parameter that serves to summarize both the overpotential and turnover frequency (catalytic current) of an electrocatalytic reaction independent of mechanistic details. This single parameter allows one to compare a variety of catalysts that transform a given substrate to the same product. Ni₃Al catalytic efficiency parameter for 1-propanol generation is calculated to be 0.5 ± 0.1%. This is comparable to the catalytic efficiency parameter for Torelli *et al.*'s Ni-Ga thin film in the generation of ethane (0.44%; based on maximum Faradaic efficiency), their major C2 product.

Furthermore, it is well established that copper electrodes suffer from instability in solution and excessive overpotential requirements for the formation of higher order organic products, making their usage to-date impractical. Ni₃Al, on the other hand, is stable in aqueous solution over the time scale explored here. This work shows that Ni₃Al generates electroreduced products from CO₂ continuously over a period of four to five days. Scanning electron microscopy confirms that the thin film is robust and, as demonstrated by the small amount of material loss observed, withstands exposure to electrochemical conditions while maintaining initial efficiencies for CO₂ reduction. This finding is supported by post-electrolysis XPS analysis demonstrating that the electrode surface composition remains unchanged during electrochemical CO₂ reduction.

The Ni₃Al thin film on glassy carbon reported here is the first copper-free, heterogeneous electrocatalyst capable of generating C₃ products, including 1-propanol and acetone, from CO₂ starting material, and its Faradaic efficiencies for 1-propanol generation are competitive with those achieved on most copper electrodes. Ultimately, these significant factors suggest that heterogeneous catalysts comprised of metals other than copper may generate highly reduced products from CO₂ whose identities, Faradaic efficiencies, selectivities, or overpotentials rival or exceed those achieved on copper catalysts.

### Methods

Thin film Ni₃Al alloys were synthesized as previously described.¹⁹ Briefly, aqueous solutions of 0.052 M nickel(II) nitrate hexahydrate and 0.036 M aluminum(III) nitrate nonahydrate were combined in appropriate ratios to achieve the Ni₃Al stoichiometry. In 0.1-mL increments, 0.5-mL portions of the nickel-aluminum nitrate solution were drop-casted onto glassy carbon pieces that had been set on a hot plate and heated to 150 °C. After drop-casting, the substrates remained on the hot plate for 15 min until the solution completely evaporated, revealing green surface films. The substrates were then placed in alumina boats and loaded into either a Lindberg/Blue M or Carbolite Quartz Tube Furnace under 95% Ar/5% H₂ gas flow. The furnace was ramped at a rate of 3 °C/min to 700 °C, where it rested for 5 h.

Electrodes were prepared by affixing a coiled copper wire to the glassy carbon substrate using conducting silver epoxy, extending the length of copper wire through a glass tube, and sealing both ends of the tube using insulating epoxy. It was critical that the insulating epoxy was also used to completely cover the silver epoxy and copper wire attached to the substrate. In some experiments, the top of a film-deposited substrate was wrapped in copper tape and held using an alligator clip attached to copper wire similarly threaded through a glass tube sealed with insulating epoxy. Comparable amounts of charge were passed in electrochemical experiments featuring the two types of electrode preparations.

Electrochemical experiments were performed using CH Instruments 760 and 1140 potentiostats. Cyclic voltammetry experiments were completed in a three-neck round-bottom flask using the Ni₃Al film on glassy carbon as the working electrode referenced to Ag/AgCl and a Pt mesh counter electrode in 0.1 M K₂SO₄ at pH 4.5. Bulk electrolysis experiments were undertaken in the same electrolyte solution (with the exception of pH dependence experiments, which utilized K₂SO₄ buffered with KHCO₃/CO₂) using custom electrolysis cells with gas-tight ports for the above electrodes. In these experiments, the Pt mesh counter electrode was situated in a fritted gas dispersion tube to separate the reduction reaction at the cathode from oxidation processes at the anode, and a stir bar was employed. The reaction solutions were purged with CO₂, CO, or Ar for 20 min prior to experimental or control trials; experiments using ¹³CO₂ were not completely purged with the starting material, resulting in a small amount of ¹²CO₂ contamination that could be quantified by ¹H-NMR. Bulk electrolysis experiments were performed over intervals of at least 4 h, during which time the headspace was sampled every 20 min and the electrochemical solution was sampled every 60 min. During and after bulk electrolysis experiments, both the solution and headspace were sampled for products using ¹H- or ¹³C-NMR (referenced to 1,4-dioxane internal standard) and gas chromatography, respectively.

### EXAMPLE 2 - Cr₂O₃-Ga₂O₃ Electrocatalytic Reduction of CO₂ to Oxalate

In this example, an electrode composed of a chromium oxide-gallium oxide thin film on glassy carbon is employed to transform CO₂ to oxalate in water. To our knowledge, this is the first heterogeneous electrocatalyst system capable of transforming CO₂ to oxalate in water, introducing new possibilities for catalyst discovery and tangible opportunities for the energy efficient conversion of CO₂ to a chemical feedstock containing more than one carbon.

Thin films of Cr-Ga (3:1 ratio) on glassy carbon solid supports were synthesized using a drop-casting and thermal reduction method adapted from Torelli et al, Nickel-gallium-catalyzed electrochemical reduction of CO2 to highly reduced products at low overpotentials. ACS Catal. 6, 2100-2104 (2016). Powder X-ray diffraction (XRD; FIG. 5A) coupled with energy-dispersive X-ray spectroscopy suggested that the bulk films were comprised of Cr₂O₃ and Ga₂O₃ in the desired 3:1 stoichiometry. Surface compositions were analyzed by X-ray photoelectron spectroscopy (FIG. 5B), which pointed to an oxidized surface comprised of mostly Cr(III), matching the bulk, and Ga oxides. Scanning electron microscopy (FIG. 1A) indicated that Cr₂O₃-Ga₂O₃ films were comprised of discontinuous platelets scattered across the glassy carbon surface, not unlike alternative bimetallic systems similarly synthesized.

Initial bulk electrolysis experiments were conducted using a Pt mesh counter electrode and 0.1 M KCl electrolyte (pH 4.1 after CO₂ purging). Applying a potential of -1.38 V vs. Ag/AgCl to an electrochemical cell purged with ¹³CO₂ induced generation of CO and H₂, sampled by gas chromatography, as well as oxalate, formate and methanol, detected in the liquid phase by ¹H and ¹³C-NMR. A high-intensity peak at 161 ppm overshadowed formate, methanol, and residual CO₂ signals and was assigned to oxalate. To confirm this product assignment, a sample of the electrolyzed solvent which had been treated with HCl to remove any carbonate present was mixed with calcium bromide, causing precipitation of a white solid which was isolated by vacuum filtration and examined by infrared (IR) spectroscopy (FIG. 6). Only IR transitions associated with calcium oxalate were observed.

In order to optimize the Cr₂O₃-Ga₂O₃ system for oxalate production, pH, electrolyte, potential dependence, and stoichiometric studies were undertaken. Gravimetric determination of oxalate is well established and was found to be quantitative in the present study when a 1 M calcium bromide solution was utilized on post electrolysis samples. Standard curves were employed for quantifying CO/H₂ and formate/methanol using gas chromatography and ¹H-NMR, respectively.

All pH-varying experiments were conducted at an applied potential of -1.38 V vs. Ag/AgCl and used CO₂-saturated KCl electrolyte (buffered with KHCO₃ for pH > 4; adjusted with HCl for pH < 4; 0.1 M concentration). As shown in FIG. 7, the Cr₂O₃-Ga₂O₃ system is only slightly sensitive to solution pH, since statistically equivalent oxalate Faradaic efficiencies were achieved at pH 4.1 and 5.1, while pH 6.1 yielded slightly inferior results. Markedly lower Faradaic efficiencies at pH 7.1 suggest that carbonate is not involved in oxalate production, as these experiments contained the highest original concentration of KHCO₃ buffer. Charge balance was achieved in all cases by H₂ generation.

In separate experiments, the electrolyte anion was varied (i.e., KCl, KBr, and KI were compared), since other researchers have reported that CO₂ reduction product selectivity can be highly electrolyte dependent. However, in the Cr₂O₃-Ga₂O₃ system, carbon-containing products did not exhibit this dependence. Subsequent experiments therefore utilized CO₂-saturated, pH 4.0 KCl, because this pH maximized total Faradaic efficiency for carbon-containing products compared to H₂. Furthermore, bulk solution pH consistently rose to 4.5-5.0 by the end of electrolysis (when initial pH = 4.1), and as shown in Fig. 7, maximum oxalate Faradaic efficiencies would still be achieved at these final pH conditions.

Subsequently, potential dependence experiments were conducted using the optimized electrolyte conditions. Notably, all potentials examined resulted in some oxalate generation, despite being significantly more positive than the thermodynamic potential required for one-electron reduction of CO₂ to CO₂˙⁻, the intermediate that has historically been invoked for the conversion of CO₂ to oxalate. The resulting Faradaic efficiencies, displayed in Fig. 8, suggest that the Cr₂O₃-Ga₂O₃ system is more sensitive to applied potential than pH. Additionally, the two major carbon-containing products, oxalate and CO, reached maximum efficiencies at different potentials. An electrode potential of -1.48 V vs. Ag/AgCl (630 mV more positive than E° for reducing CO₂ to CO₂˙⁻) was determined to be the optimal potential for oxalate production.

A cell employing 0.1 M KCl (pH 4.0) at a potential of -1.48 V vs. Ag/AgCl, generated Faradaic efficiencies for oxalate, CO, formate, and methanol of 59 ± 3%, 8.1 ± 0.7%, 0.16 ± 0.02%, and 0.15 ± 0.02%, respectively. Materials characterization post-electrolysis suggested that Cr₂O₃-Ga₂O₃ system continued to be chemically and physically stable. XPS analysis revealed only subtle changes in surface composition. Surface Cr remained more than 99% Cr(III), in agreement with the Cr Pourbaix diagram. Still, Ga metal did not make up the majority of the sample, but its XPS spectrum largely resembled its pre-electrolysis analog, confirming a stable surface. SEM imaging indicated that the thin film incurred only slight erosion at platelets' edges during electrolysis, while EDX showed that the 3:1 Cr:Ga stoichiometry was maintained. A single Cr₂O₃-Ga₂O₃/glassy carbon electrode could transform CO₂ continuously for more than 10 days (the longest time period studied), suggesting an attractive catalytic lifetime.

### Determination of reaction intermediates en route to oxalate

The Cr₂O₃-Ga₂O₃ film on glassy carbon is a promising catalyst due to its high oxalate Faradaic efficiency, good stability, and, perhaps most interestingly, its ability to perform the electrochemical transformation in water. At the applied potentials studied here, ranging from 530 to 930 mV more positive than the E° required for CO₂˙⁻ generation, CO₂ reduction to oxalate cannot occur through a CO₂˙⁻ intermediate, which means a pathway as-yet unreported for the electrochemical CO₂-to-oxalate transformation must be at play. While prior studies often rely on the supposition of a CO₂˙⁻ intermediate, calculations have been performed evaluating a homogeneous catalytic system, consisting of a dinuclear Cu complex in acetonitrile solvent, that explicitly refute a CO₂˙⁻-dependent pathway in that case. To determine whether any of the alternative CO₂ reduction products serve as intermediates en route to oxalate, a series of electrolysis experiments were performed, which replaced the CO₂ feedstock with CO, formate, methanol, or combinations of these carbon-containing compounds.

Ultimately, during electrolysis experiments conducted using the optimized pH, electrolyte, and potential plus ¹³CO and methanol (rather than CO₂), oxalate was produced, as confirmed by precipitation with calcium bromide as well as ¹³C-NMR. This ¹³CO experiment, which used ¹²C-methanol, also verified that CO was incorporated into the oxalate product. The opposite labeling experiment, using ¹²CO and ¹³C-methanol, was also undertaken, resulting in no ¹³C-NMR signal even though calcium oxalate was precipitated out of solution. Therefore, methanol is not incorporated into the product. Significantly, supplying Cr₂O₃-Ga₂O₃ with either CO or methanol, rather than both, does not result in an oxalate end product; both species are required even though only the CO ends up in the reaction product. Rather than a CO₂˙⁻-dependent pathway, Cr₂O₃-Ga₂O₃ production of oxalate therefore appears to rely on CO and methanol, which it can first generate from CO₂.

The incorporation of CO and use of short-chain alcohols in oxalate generation is not unprecedented, although it has not previously been accomplished using a CO₂ starting material. Large-scale manufacture of oxalate is frequently accomplished by oxidative carbonylation of small alcohols to achieve diesters of oxalic acid, followed by hydrolysis to attain the oxalate product. This reaction consumes O₂ to re-oxidize the catalyst, which can be a two-component metal system, such as Pd plus FeCl₂ or CuCl₂.

FIG 9 illustrates Faradaic efficiencies of carbon-containing products. While oxalate generation is generally suppressed at high KCl concentrations, low CO and high formate Faradaic efficiencies contribute to decreased oxalate production at low KCl concentrations. Electrolyses were performed at -1.48 V vs. Ag/AgCl. In feedstock experiments, formate was shown to be a competitor of, rather than intermediate contributing to, oxalate production.

Cr₂O₃-Ga₂O₃ methods of generating oxalate exhibit critical mechanistic differences with oxidative carbonylation processes, which could make Cr₂O₃-Ga₂O₃ a more attractive option for oxalate synthesis. Ultimately, the Cr₃Ga catalyst introduces a new and practical means of generating oxalate from CO₂, but it also demonstrates that electrochemical routes excluding a CO₂˙⁻ intermediate are not only possible but can operate both in aqueous environments and at much lower applied potentials than previously thought.

Such a departure from the previously accepted mode of CO₂ reduction to oxalate invites a question about the roles of the metals within the Cr₂O₃-Ga₂O₃ catalyst. To answer that question, the pure metal films as electrocatalysts were first examined. At -1.48 V vs. Ag/AgCl (pH 4.0 KCl), films of Cr on glassy carbon generated modest amounts of CO, formate, and methanol from CO₂, while the activity of Ga films was dominated by CO production at around 40% Faradaic efficiency. Regardless, plain Ga thin films converted about 20% of the CO₂ in the system to carbonate, observable on the surface post-electrolysis by XPS, while Cr's carbonate production was more limited. As thin films, neither metal alone could produce oxalate from CO₂, confirming the importance of having both metals present.

A clear need for both Cr and Ga implies that an optimal Cr:Ga stoichiometry exists for maximizing oxalate production. To determine this stoichiometry and gain additional insight into the role of each metal, a range of stoichiometries spanning from 100% Cr to 100% Ga were synthesized as thin films on glassy carbon and analyzed for their performance as CO₂ reduction electrocatalysts. All experiments were conducted at -1.48 V vs. Ag/AgCl in 0.1 M KCl (pH 4.05) for comparison to the optimized oxalate outcome for Cr₂O₃-Ga₂O₃.

The trends in carbon-containing product generation based on Cr:Ga stoichiometry are displayed in Fig. 10. Cr₂O₃-rich stoichiometries corresponded to lower overall quantities of non-oxalate products compared to Ga-rich variants, but, most notably, Faradaic efficiencies for CO (essential for oxalate generation) reached their lowest values at the highest percentages of Cr. The highest Faradaic efficiency for oxalate was obtained at the original 3Cr:1Ga stoichiometry. When considering the product trends in FIG. 10, it seems that optimal oxalate generation requires ideal combinations of CO/methanol production and formate suppression. Some critical quantity of Cr is needed to ensure that oxalate is produced efficiently, but excess Cr prevents adequate generation of CO, which decreases oxalate Faradaic efficiencies. Complementarily, Ga seems to be the major CO-generating component of the system. In combination, these factors make Cr₂O₃-Ga₂O₃ one preferred embodiment for oxalate production, with the recognition that oxalate production can be achieved with other electrode compositions, systems and methods described herein. Other alloys and/or oxides thereof exhibiting the mechanistic requirements described herein may be employed for oxalate production.

The ability of the Cr₂O₃-Ga₂O₃ thin film on glassy carbon to generate oxalate from CO₂ in water makes it a landmark example of heterogeneous CO₂ electroreduction, as previous studies of this conversion were confined to use of nonaqueous electrolytes and applied potentials reflective of a CO₂˙⁻ intermediate. With optimal electrolysis conditions of pH 4.0 aqueous KCl and -1.48 V vs. Ag/AgCl, the pathway used to generate oxalate by this system must not include CO₂˙⁻ coupling. Instead, CO₂ is reduced to CO and methanol, which are then used to produce oxalate.

Oxalate Faradaic efficiencies of 59 ± 3% and initial lifetime studies exceeding 10 days of continuous use show the potential for Cr₂O₃-Ga₂O₃ as a candidate catalyst for a new industrial oxalate process, especially because it achieves the desired end product using aqueous solution, atmospheric pressure, and CO₂ starting material.

### Nature of Cr-Ga Surface Sites Active in CO₂ Reduction

Notably, the reactant experiments that initially pointed to oxalate-generating roles for CO and methanol did not implicate an important role for formate, which has been indicated as a competitor of oxalate production in the literature. With a Cr-Ga electrode, use of a formate feedstock resulted in only trace amounts of methanol and failed to generate oxalate. This result suggested that distinct active sites may exist for generation of formate and CO-derived products, including oxalate. Further support for this prediction was provided by electrolyte dependence studies. While experiments varying the electrolyte anion (i.e., KCl, KBr, KI, K₂SO₄, and KH₂PO₄) failed to exhibit significant differences in the distribution of products, a stark dependence was noted when varying the electrolyte cation.

Use of LiCl or NH₄Cl electrolytes (0.1 M) and -1.48 V vs. Ag/AgCl applied potential resulted in similar product distributions and efficiencies as those recorded for KCl. However, analogous experiments using CsCl, (CH₃)₄NCl ((TMA)Cl), and CaCl₂ electrolytes failed to generate any detectable quantities of oxalate, and CO Faradaic efficiencies were also reduced. (TMA)Cl supporting electrolyte increased the Faradaic efficiency of formate to 7.7 ± 0.4%, compared to the 0.16 ± 0.02% value achieved using optimal oxalate-generating conditions (0.1 M KCl). These cation-dependence results are summarized in Table 2.

Furthermore, Cr-Ga electrodes previously used in (TMA)Cl experiments did not regain their oxalate-generating ability when re-introduced into a KCl-containing electrolyte. This KCl electrolyte was subjected to ¹H-NMR after electrolysis, and the resultant spectrum exhibited an overwhelming signal from TMA⁺, which must have come from the Cr-Ga surface. TMA⁺ had therefore chemisorbed to the catalyst during prior electrolyses, likely contributing to inhibition of oxalate generation in those and subsequent experiments. Formate generation remained higher than usual in these trials.

Exacerbation of formate production when oxalate generation is suppressed further supports the proposal that at least two surface active sites are present in the Cr-Ga catalyst: one for CO and CO-derived productions and a second for formate. Moreover, chemisorption of TMA⁺ onto the Cr-Ga surface suggests that a surface anion is present, while lack of oxalate production in the presence of cations having few waters of hydration (TMA⁺ and Cs⁺) or strong anion-binding capacity (Ca²⁺) hints that this surface anion is critical to CO/oxalate generation. To probe this theory, the Cr-Ga system (0.1 M KCl, -1.48 V vs. Ag/AgCl) was treated with 15 mM NaCN prior to electrolysis, anticipating that the Lewis-basic, anionic CN⁻ ligand would bind specifically to a Lewis-acidic, non-anionic surface site. Indeed, after performing electrolysis with this modified system, CO, oxalate, and methanol were detected in typical yields, while no formate was produced. Thus, it appears that the CN⁻ ligates the formate-generating active site, simultaneously demonstrating that this site is (A) chemically distinct from the CO-generating site and (B) not anionic in character. This experiment, combined with the cation-dependence data, strongly suggests that Cr-Ga contains two types of electrocatalytic surface sites for CO₂ reduction: an anionic site leading to CO-derived products and a non-anionic site that produces formate.

### Materials and Methods

### Materials

Chromium(III) nitrate nonahydrate (≥ 99.99%), gallium(III) nitrate hydrate (99.9%), KHCO₃ (99.7%), oxalic acid (≥ 99%), NH₄Cl (99.998%), (CH₃)₄NCl ((TMA)Cl; ≥ 98%), NaCN (97%), methanol (≥ 99.9%), ¹³C-methanol (99 at% ¹³C), formic acid (≥ 98%), 1,4-dioxane (99.8%), acetonitrile (99.8%), ethanol (≥ 99.8%), isopropanol (≥ 99.7%), ¹³CO₂(99 at% ¹³C), ¹²CO (¹³C-depleted), and ¹³CO (99 at% ¹³C) were obtained from Sigma-Aldrich. KCl, KBr, KI, K₂CO₃, K₂SO₄, KH₂PO₄, LiCl, CsCl, CaCl₂, and HCl, all ACS grade, were purchased from EMD Chemicals, and calcium bromide (99.5%) was obtained from Alfa Aesar. Ar, CO₂, CO, 95% Ar/5% H₂, and 50% CO/50% H₂ gases and mixtures were ordered from AirGas. Glassy carbon plates (GLAS 11; 25 x 25 x 3 mm; Structure Probe Inc.) were cut in half lengthwise prior to use. Conducting silver and Loctite Hysol insulating epoxies were purchased from Epo-Tek and Grainger, respectively. All chemicals were used as received except for methanol and formic acid for standard curves, 1,4-dioxane for NMR internal standards, and HCl, all of which were diluted prior to use.

### Methods

Synthetic procedures to create Cr-Ga thin films of various stoichiometries are described. Aqueous solutions of 0.052 M chromium(III) nitrate nonahydrate and 0.036 M gallium(III) nitrate hydrate were mixed to achieve the desired Cr:Ga ratio. Glassy carbon pieces were heated to -120 °C on a hotplate, and 0.1-mL samples of the Cr-Ga nitrate solution were drop-casted onto them. After the solution evaporated completely, the glassy carbon pieces were placed in an alumina boat and loaded into either a Lindberg/Blue M or Carbolite Quartz Tube Furnace. The furnace was ramped at a rate of 3 °C/min to 700 °C under 95% Ar/5% H₂ gas flow; it rested at this state for 5 h prior to cooling to room temperature at a rate of -3 °C/min. Resulting Cr-Ga films were olive green in color, with Cr-rich stoichiometries tending toward kelly green and Ga-rich stoichiometries tending toward gray.

Electrodes were prepared in one of two fashions. One electrode configuration involved connecting copper wire to the glassy carbon support using conducting silver epoxy, feeding the wire through a glass tube, and covering both ends of the tube (including any exposed copper or silver) with insulating epoxy. The second configuration featured the same general setup, but the copper wire was attached to an alligator clip, which could then be used to reversibly hold glassy carbon pieces whose tops had been wrapped in copper tape. Experiments using both electrode configurations yielded identical results, both in terms of charge passage and product distribution.

Electrochemical experiments were conducted using CH Instruments 760 and 1140 potentiostats. Bulk electrolysis experiments utilized custom electrochemical cells with gas-tight ports for the working, Pt mesh counter (situated in a gas dispersion tube), and Ag/AgCl reference electrodes. The electrolyte was continuously stirred. Unless otherwise noted, 0.1 M KCl was used as the electrolyte, and it was buffered with KHCO₃ to achieve CO₂-saturated pH values > 4 or adjusted with 0.01 M HCl for values < 4. Electrolyte solutions were purged with CO₂ for 30 min prior to experimentation. In experiments without CO₂ (i.e., CO, formic acid, methanol, or combinatorial feedstocks), the pH was adjusted to the appropriate, CO₂-analogous value. The majority of electrolyses were conducted at pH 4.1, and post-electrolysis measurements indicated that the final solution pH was consistently between 4.5 and 5.0. Experiments using ¹³CO₂, ¹³CO, and ¹²CO (¹³C-depleted) were not completely purged with the respective gas.

Electrolysis experiments were performed until 30-40°C charge had passed, unless the experiment was meant to determine catalyst lifetime. The solution and headspace of electrochemical cells were sampled for liquid and gaseous products by ¹H-NMR (referenced to 1,4-dioxane internal standard) and gas chromatography, respectively, both during and after bulk electrolysis. Oxalate was detected by ¹³C-NMR and quantified by precipitation of the calcium salt.

### Cr-Ga Thin Film Characterization

The compositions and morphologies of Cr-Ga films were analyzed by a variety of materials characterization techniques. Powder X-ray diffraction was performed using a Bruker D8 Advance diffractometer with 0.083° step size and CuKα radiation. XRD samples either remained on the glassy carbon support or were scraped from the surface; resulting patterns were identical, except that scraped samples exhibited significantly less carbon intrusion and were therefore selected for presentation herein. Thin film morphology and additional bulk composition data were obtained using a FEI XL30 FEG-SEM equipped with EVEX EDS detector. SEM images and EDX spectra were obtained using a 5 or 10 keV electron beam with a 10-15 mm working distance. XPS spectra were collected using a ThermoFisher K-Alpha X-Ray Photoelectron Spectrometer set to 20 eV pass energy and 50 ms dwell time. Resulting data were analyzed using the Thermo Scientific Avantage Data System and CasaXPS software. Materials characterization was conducted before and after electrochemistry in designated experiments.

### Product Analysis

Formate and methanol were detected by ¹H-NMR after combining 530 µL electrolyte with 60 µl D₂O and 10 µL 1,4-dioxane (10 mM); the latter served as an internal standard. In ¹³C-NMR experiments (used primarily to detect oxalate), only 1 µL 1,4-dioxane (10 mM) was added. A Bruker Avance III 500 MHz NMR Spectrometer with cryoprobe detector was used for all NMR experiments, and the experiments incorporated a custom water suppression method to permit sampling of aqueous electrolyte solutions. Formate and methanol were quantified using 5-point calibration curves for ¹H-NMR, while oxalate was visualized qualitatively by a large ¹³C-NMR signal (in experiments utilizing ¹³C-labeling) in the 160-170 ppm range.

Oxalate was quantified by first treating a sample of the electrolysis solution with 1 M HCl (to remove any carbonate byproduct) and then adding 1 M calcium bromide solution, which resulted in the precipitation of calcium oxalate. The calcium oxalate sample was dried in an oven at 105 °C overnight and then massed; this mass was used to calculate the total quantity of oxalate. IR spectra of calcium oxalate samples were obtained using a Thermo Diamond Smart Orbit IR Spectrometer set at 1 cm⁻¹ resolution. The carbonate byproduct could be quantified by finding the difference in mass between two electrolysis samples, one treated with HCl and the other untreated prior to calcium bromide addition; the difference in mass was attributed to calcium carbonate, which was then calculated as a percentage of the total CO₂ in solution (based on the electrolyte volume unique to each experiment). Calcium carbonate was also examined by IR spectroscopy. Experimental calcium oxalate and calcium carbonate samples were compared to control compounds made by combining calcium bromide and either oxalic acid or K₂CO₃ in aqueous solution.

Headspace samples were analyzed by gas chromatography for gaseous products. CO was measured using a HP6890 Gas Chromatograph fitted with a Molsieve 5A PLOT capillary column (Agilent) and TCD. The sampling method was a 5-min, 60 °C isotherm with He flow gas. An SRI 8610C Gas Chromatograph with Ar flow, which also used a Molsieve column and TCD, was run for a 7-min isotherm at 80 °C to detect H₂. CO and H₂ were quantified using 30-point calibration curves having R² values ≥ 0.99. The headspace was also sampled following ¹³CO₂ electrolyses using a KBr-terminated gas cell and Nicolet iS50 FT-IR Spectrometer with 1 cm⁻¹ resolution; this confirmed that the CO product was derived from CO₂. Faradaic efficiencies for all products, gaseous and liquid, were calculated based on the charge passed during each experiment as well as the product quantities determined by gas chromatography, ¹H-NMR, or calcium bromide precipitation. Catalytic efficiencies were calculated based on the following equation: $Catalytic efficiency = \frac{Faradaic efficiency}{\left(1+\frac{overpotential}{{{E}^{° ′}}_{product}}\right)} \times 100 %$

Various embodiments of the invention have been described in fulfillment of the various objects of the invention. It should be recognized that these embodiments are merely illustrative of the principles of the present invention. Numerous modifications and adaptations thereof will be readily apparent to those skilled in the art without departing from the scope of the invention.

## Claims

1. A system for providing oxygenated organic products comprising:
an electrochemical cell including an electrolyte solution comprising CO₂,
and an electrode comprising a mixture of metal oxides wherein the mixture of metal oxides comprises chromium oxide and gallium oxide,
the electrode having an electrocatalytic site for reduction of CO₂ to CO, wherein the oxygenated organic products are derived from the CO.

2. The system of claim 1, wherein the ratio of chromium to gallium is 3:1 .

3. The system of claim 1, wherein the electrolyte solution has an acidic pH.

4. A method for providing oxygenated organic products comprising the use of a system as claimed in any preceding claim, the method comprising reducing CO₂ to CO at the electrocatalytic site on the electrode; and
deriving the oxygenated organic products from the CO.

5. A method as claimed in Claim 4 wherein the oxygenated organic products comprise oxalate.

## Patentansprüche

1. System zur Bereitstellung von sauerstoffhaltigen organischen Erzeugnissen, bestehend aus:
eine elektrochemische Zelle mit einer Elektrolytlösung, die CO₂ enthält,
und eine Elektrode, die ein Gemisch von Metalloxiden umfasst, wobei das Gemisch von Metalloxiden Chromoxid und Galliumoxid umfasst,
die Elektrode weist eine elektrokatalytische Stelle zur Reduktion von CO₂ zu CO auf, wobei die sauerstoffhaltigen organischen Produkte aus dem CO abgeleitet sind.

2. System nach Anspruch 1, wobei das Verhältnis von Chrom zu Gallium 3:1 beträgt.

3. System nach Anspruch 1, wobei die Elektrolytlösung einen sauren pH-Wert aufweist.

4. Verfahren zur Bereitstellung sauerstoffhaltiger organischer Produkte, umfassend unter Verwendung eines Systems nach einem der vorhergehenden Ansprüche, wobei das Verfahren die Reduktion von CO₂ zu CO an der elektrokatalytischen Stelle an der Elektrode umfasst; und
die sauerstoffhaltigen organischen Produkte aus dem CO ableiten.

5. Verfahren nach Anspruch 4, wobei die sauerstoffhaltigen organischen Produkte Oxalat umfassen.

## Revendications

1. Système de fourniture de produits organiques oxygénés comprenant :
une pile électrochimique comprenant une solution d'électrolyte comprenant du CO₂, et électrode comprenant un mélange d'oxydes métalliques, le mélange d'oxydes métalliques comprenant de l'oxyde de chrome et de l'oxyde de gallium,
l'électrode ayant un site électrocatalytique pour la réduction du CO₂ en CO, dans lequel les produits organiques oxygénés sont dérivés du CO.

2. Système selon la revendication 1, dans lequel le rapport entre le chrome et le gallium est de 3:1 .

3. Système selon la revendication 1, dans lequel la solution d'électrolyte a un pH acide.

4. Procédé d'obtention de produits organiques oxygénés comprenant l'utilisation d'un système selon l'une quelconque des revendications précédentes, le procédé comprenant la réduction du CO₂ au CO au site électrocatalytique sur l'électrode ; et dérivant les produits organiques oxygénés du CO.

5. Procédé selon la revendication 4, dans lequel les produits organiques oxygénés comprennent de l'oxalate.
